# EUROPEAN PATENT SPECIFICATION

(11) **EP 0 510 249 B1**
(45) Date of publication and mention of the grant of the patent: **08.03.2000**
(21) Application number: 91114828.6
(22) Date of filing: 03.09.1991
(51) Int. Cl.: C21D 8/04

(54) **Cold reduced non-aging deep drawing steel and method for producing**
Kaltverformtes und nichtalterndes Tiefziehblech aus Stahl und Herstellungsverfahren
Tôle en acier formé à froid pour emboutissage avec une résistance au vieilissement et procédé de fabrication

(30) Priority: 25.06.1991 US 720966; 23.04.1991 US 690142
(43) Date of publication of application: 28.10.1992
(73) Proprietor: AK Steel Corporation, Middletown, Ohio 45043 (US)
(72) Inventor: Rollin E. Hook, Dayton Ohio 45431 (US)
(74) Representative: Beetz & Partner Patentanwälte

(56) References cited:
- US-A- 3 798 076
- US-A- 3 959 029
- US-A- 4 116 729
- US-A- 4 145 235
- US-A- 4 473 411
- US-A- 4 478 649
- US-A- 4 627 881
- US-A- 4 698 102
- ISIJ INTERNATIONAL, vol. 30, no. 9, 1990, TOKYO,JP pages 764 - 772 K.USHIODA ET AL.

## Description

This invention relates to a method of producing an aluminum killed steel, particularly, a low manganese, batch annealed steel produced from a slab having a reduced hot rolling temperature.

It is well known deep drawing steels are characterized as requiring a very high average plastic strain ratio(rₘ) of 1.8 or more. Average plastic strain ratio is defined as ${\text{r}}_{\text{m}} {\text{= (r}}_{\text{0}} {\text{°+ r}}_{\text{90}} {\text{° +2r}}_{\text{45}} \text{°)/4}$. High rₘ values have been achieved by adding various carbide and/or nitride formers, e.g., Ti, Cb, Zr, B, and the like, to steel melt compositions. However, addition of these elements to a melt to produce deep drawing steel is undesirable because of the added alloy costs. It also is known aluminum killed steel having an equiaxed grain structure with similar high rₘ values can be produced by continuous annealing if aluminum nitride is precipitated prior to cold reduction. Batch annealed, aluminum killed steel having an elongated grain structure can develop rₘ values of about 1.8 by precipitating aluminum nitride during the slow heatup prior to the onset of recrystallization during annealing. Unlike for batch annealing, aluminum nitride will not precipitate prior to recrystallization during continuous annealing to form high rₘ values because the heating rate is too rapid. Precipitation of aluminum nitride prior to cold reduction to produce high rₘ values for continuously annealed aluminum killed steel is accomplished by using a high coiling temperature after hot rolling or by reheating a relatively cold slab to a temperature insufficient to re-dissolve aluminum nitride precipitated during cooling of the slab following casting.

The following prior art discloses cold reduced, aluminum killed steel produced by continuous annealing. The US-A-4,145,235 discloses a process for producing a low manganese, aluminum killed steel having high rₘ values by hot coiling a sheet at a temperature no less than 735°C after hot rolling. Values for rₘ up to 2.09 after continuous annealing are disclosed. The US-A 4,478,649 discloses a process for direct hot rolling a continuously cast aluminum killed steel slab without reheating the slab. The as-cast slab is hot rolled prior to the slab cooling to a temperature below Ar₃ thereby avoiding precipitation of aluminum nitride. Aluminum nitride is precipitated prior to continuous annealing by hot coiling the sheet at a temperature of at least 780°C after hot rolling. The US-A 4,698,102 discloses using slab temperatures for aluminum killed steel less than 1240°C so that aluminum nitride precipitated during cooling of the slab following casting is not re-dissolved prior to hot rolling. Coiling temperatures after hot rolling of 620-710°C are disclosed to precipitate any remaining solute nitrogen prior to continuous annealing. The US-A 4,116,729 discloses cooling a continuously cast aluminum killed steel slab to within the temperature range of 650°C to Ar₃ for at least 20 minutes to precipitate aluminum nitride. The slab then is reheated to 950-1150°C for hot rolling without re-dissolving the aluminum nitride. Values for rₘ up to 1.6 after continuous annealing are disclosed. The US-A 4,627,881 discloses a process for producing high rₘ values in continuously annealed aluminum killed steel by controlling the nitrogen to no greater than 0.0025% and the phosphorus to no greater than 0.010% with the sum of phosphorus plus five times the nitrogen no greater than 0.020%. Slabs were reheated and hot rolled within the temperature range of 1050-1200°C. The hot rolled sheet was coiled at a temperature of less than 650°C. Cold reduced, continuously annealed sheet had rₘ values up to 2.1. It also is known continuously annealed aluminum killed steel having high rₘ values can be produced by increasing the soluble aluminum in the melt. The US-A 3,798,076 discloses an aluminum killed steel having .13 to .33% soluble aluminum and rₘ values up to 1.91 after continuous annealing.

It is known aluminum killed steel having similar high rₘ values can be produced by batch annealing. The US-A 3,959,029 discloses using conventional slab hot rolling practice so as not to precipitate aluminum nitride, i.e., keep nitrogen in solution, prior to batch annealing. Values for rₘ up to 2.23 were disclosed for a non-aging, aluminum killed steel by decarburizing a cold reduced sheet during annealing to less than .01 % carbon.

The JP-A-57-70237 discloses a method of producing deep rolled steel sheets having superior deep drawability. The used steel containing ≤ 0.08 % C, ≤ 0.08 % Si, 0.05 to 0.35 % Mn, ≤ 0.07 % S, 0.01 to 0.12 % Al, 0.002 to 0.015 % N and the remainder Fe and impurities will be heated to a temperature ≥ 1100 °C and then finishing annealed at a temperature ≥ the Ar₃-point. After a usual cold rolling the steel strip is coiled at a temperature of 300 to 500 °C.

The US-A-4 473 411 - as nearest prior art-discloses a batch annealed aluminum killed steel having rₘ values up to 1.85. The sheet was produced from a slab using conventional (1260°C slab drop-out temperature) hot rolling practice having .12-.24% manganese that was hot rolled without precipitating aluminum nitride. The hot rolled sheet was cold reduced and its cold spot temperature carefully controlled during annealing to develop high rₘ values.

Addition of carbide and/or nitride forming elements to a melt to produce non-aging deep drawing steel is undesirable because of the alloy costs. Melt processing techniques, i.e., vacuum degassing, ladle stirring, fluxing, and the like, required to reduce residual carbon, nitrogen or phosphorus are expensive. Using elevated coiling temperatures to produce non-aging, deep drawing, aluminum killed steel is undesirable because of uneven cooling rates and the scale formed on the hot rolled sheet during cooling from the elevated coiling temperature is more difficult to remove. Special decarburizing annealing cycles to produce non-aging, deep drawing, aluminum killed steel is undesirable because of added costs. Accordingly, there remains a need for an inexpensive, non-aging, deep drawing, aluminum killed steel. More particularly, there remains a need for a batch annealed, aluminum killed steel having an rₘ value of 1.8 or more that can be produced using conventional processing or using processing that does not add, and preferably reduces, cost over that of conventional processing.

This invention relates to method of producing a cold reduced, non-aging, recrystallization batch annealed steel as defined in claim 1. Said steel consists of ≤ 0.08% carbon, < 0.1% acid sol. aluminum, ≤ 0.2% manganese, all percentages by weight, the balance iron and unavoidable impurities, the steel produced from a slab hot rolled from a temperature less than about 1260°C to a sheet having nitrogen in solution. More preferably, the steel consists of carbon ≤ 0.05%, manganese < 0.20%, acid sol. aluminum 0.03-0.08%, total nitrogen 0.003-0.007% wherein % acid sol. aluminum x % total nitrogen is no greater than about 5 x 10⁻⁴. Most preferably, the steel has an rₘ value of at least 2.0 after being annealed at a temperature of 538-649°C, consists of manganese ≤ 0.16%, acid sol. aluminum 0.05-0.06%, total nitrogen 0.004-0.006% wherein % acid sol. aluminum x % total nitrogen is within the range of 2 x 10⁻⁴ to 4 x 10⁻⁴ and is produced from a continuously cast slab hot rolled from a temperature less than about 1175°C.

Principal objects of the invention include producing a non-aging, deep drawing, aluminum killed steel without using melt alloying additions or without degassing, stirring or fluxing the melt to reduce residual carbon, nitrogen, or phosphorus to very low amounts.

Another object of the invention includes producing a non-aging, deep drawing, aluminum killed steel without using an elevated coiling temperature after hot rolling.

A further object of the invention includes producing a non-aging, deep drawing, aluminum killed steel without using a special batch annealing cycle such as decarburization.

The non-aging, cold reduced, recrystallization batch annealed steel sheet produced according to the invention is characterized by an elongated grain structure and an rₘ value of at least 1.8 consisting of ≤ 0.08% carbon, ≤ 0.1% acid sol. aluminum ≤ 0.20% manganese, all percentages by weight, the balance iron and unavoidable impurities, the sheet having been produced from a slab hot rolled from a temperature less than about 1260°C to a sheet having nitrogen in solution.

Such a non-aging, cold reduced, recrystallization batch annealed steel sheet can have an elongated grain structure and an rₘ value of at least 2.0 consisting of ≤ 0.05% carbon, 0.02-0.1 % acid sol. aluminum, ≤ 0.20% manganese, all percentages by weight, the balance iron and unavoidable impurities, the sheet having been produced from a continuously cast slab hot rolled from a temperature less than about 1175°C to a sheet having nitrogen in solution.

Further a non-aging, cold reduced, recrystallization batch annealed steel sheet can be characterized by an elongated grain structure and an rₘ value of at least 1.8 consisting of ≤ 0.08% carbon, ≤ 0.2% manganese, ≥ 0.01 acid sol. wt.% aluminum and nitrogen as an impurity, wherein the product of % acid sol. aluminum and % total nitrogen is ≤ 5 x 10⁻⁴, all percentages by weight, the balance iron and unavoidable impurities, the sheet having been produced from a slab hot rolled from a temperature less than about 1260°C to a sheet having nitrogen in solution.

Further a non-aging, cold reduced, recrystallization batch annealed steel sheet produced according to the invention can be characterized by an elongated grain structure and an rₘ value of at least 2.0 consisting of ≤ 0.05% carbon, 0.03-0.08% acid sol. aluminum, 0.003-0.007% total nitrogen, < 0.20% manganese, wherein the product of % acid sol. aluminum and % total nitrogen is ≤ 5 x 10⁻⁴, all percentages by weight, the balance iron and unavoidable impurities, the sheet having been produced from a continuously cast slab hot rolled from a temperature less than about 1175°C to a sheet having nitrogen in solution.

Further a non-aging, cold reduced, recrystallization batch annealed steel sheet produced according to the invention can be characterized by an elongated grain structure and an rₘ value of at least 2.0 consisting of ≤ 0.05% carbon, 0.05-0.06% acid sol. aluminum, 0.004-0.006% total nitrogen, ≤ 0.16% manganese, wherein the product of % acid sol. aluminum and % total nitrogen is within the range of 2 x 10⁻⁴ to 4 x 10⁻⁴, all percentages by weight, the balance iron and unavoidable impurities, the sheet haying been produced from a continuously cast slab hot rolled from a temperature less than about 1175°C to a sheet having nitrogen in solution.

According to another feature of the invention the method of producing a steel sheet include the steps of providing a melt consisting of ≤ 0.08% carbon, ≤ 0.1% acid sol. aluminum, ≤ 0.20% manganese, all percentages by weight, the balance iron and unavoidable impurities, casting the melt into a slab having a thickness no greater than 50 mm, hot rolling the slab having a temperature less than about 1260°C to a sheet having nitrogen in solution, descaling the hot rolled sheet, cold reducing the descaled sheet, recrystallization batch annealing the cold reduced sheet wherein the annealed sheet is non-aging, characterized by having an elongated grain structure and an rₘ value of at least 1.8.

According to another feature of the invention the method of producing a steel sheet include the steps of providing a melt consisting of ≤ 0.05% carbon, 0.02-0.1% acid sol. aluminum, ≤ 0.20% manganese, all percentages by weight, the balance iron and unavoidable impurities, casting the melt into a slab, hot rolling the slab having a temperature less than about 1175°C to a sheet having nitrogen in solution, descaling the hot rolled sheet, cold reducing the descaled sheet, recrystallization batch annealing the cold reduced sheet wherein the annealed sheet is non-aging, characterized by an elongated grain structure and has an rₘ value of at least 2.0.

According to another feature of the invention the method of producing a steel sheet include the steps of providing a slab consisting of ≤ 008% carbon, ≤ 0.2% manganese, ≥ 0.01 acid sol. wt.% aluminum and nitrogen as an impurity, wherein the product of % acid sol. aluminum and % total nitrogen is ≤ 5 x 10⁻⁴, all percentages by weight, the balance iron and unavoidable impurities, hot rolling the slab having a temperature less than about 1260°C to a sheet having nitrogen in solution, descaling the hot rolled sheet, cold reducing the descaled sheet, recrystallization batch annealing the cold reduced sheet wherein the annealed sheet is non-aging, characterized by having an elongated grain structure and an rₘ value of at least 1.8.

According to another feature of the invention the method of producing a steel sheet includes the steps of providing a melt consisting of ≤ 0.05% carbon, 0.03-0.08% acid sol. aluminum, 0.003-0.007% total nitrogen, < 0.20% manganese, wherein the product of % acid sol. aluminum and % total nitrogen is ≤ 5 x 10⁻⁴, all percentages by weight, the balance iron and unavoidable impurities, casting the melt into a slab, cooling the slab to a temperature below Ar₃ to precipitate aluminum nitride, reheating the slab to a temperature less than 1175°C to redissolve the aluminum nitride, hot rolling the slab to a sheet having a finishing temperature at least equal to Ar₃ and a coiling temperature no greater than 593°C wherein the hot rolled sheet has nitrogen in solution, descaling the hot rolled sheet, cold reducing the descaled sheet, recrystallization batch annealing the cold reduced sheet wherein the annealed sheet is non-aging, characterized by an elongated grain structure and an rₘ value of at least 2.0.

According to another feature of the invention the method of producing a steel sheet includes the steps of providing a melt consisting of ≤ 0.05% carbon, 0.05-0.06% acid sol. aluminum, 0.004-0.006% total nitrogen, < 0.20% manganese, wherein the product of % acid sol. aluminum and % total nitrogen is in the range of 2 x 10⁻⁴ to 4 x 10⁻⁴, all percentages by weight, the balance iron and unavoidable impurities, casting the melt into a slab, cooling the slab to a temperature below Ar₃ to precipitate aluminum nitride, reheating the slab to a temperature less than 1175°C to redissolve the aluminum nitride, hot rolling the slab to a sheet having a finishing temperature at least equal to Ar₃ and a coiling temperature no greater than 593°C wherein the hot rolled sheet has nitrogen in solution, descaling the hot rolled sheet, cold reducing the descaled sheet, recrystallization batch annealing the cold reduced sheet wherein the annealed sheet is non-aging, characterized by an elongated grain structure and an rₘ value of at least 2.0.

According to another feature of the invention the method of producing a steel sheet includes the steps of providing a melt consisting of ≤ 0.05% carbon, 0.05-0.06% acid sol. aluminum, 0.004-0.006% total nitrogen, ≤ 0.16% manganese, wherein the product of % acid sol. aluminum and % total nitrogen is in the range of 2 x 10⁻⁴ to 4 x 10⁻⁴, all percentages by weight, the balance iron and unavoidable impurities, casting the melt into a slab, cooling the slab to a temperature below Ar₃ to precipitate aluminum nitride, reheating the slab to a temperature of less than 1175°C to redissolve the aluminum nitride, hot rolling the slab to a sheet having a finishing temperature at least equal to Ar₃ and a coiling temperature no greater than 593°C wherein the hot rolled sheet has nitrogen in solution, descaling the hot rolled sheet, cold reducing the descaled sheet, recrystallization batch annealing the cold reduced sheet in the range of 538-649°C wherein the annealed sheet is non-aging, characterized by an elongated grain structure and an rₘ value of at least 2.0.

Advantages of the invention include a cold reduced, non-aging, recrystallization batch annealed, aluminum killed steel characterized by an elongated grain structure and an rₘ value of at least 1.8 produced by hot rolling a slab having reduced temperature thereby effecting savings in energy costs, improving yields and productivity and extending the life of a slab heating furnace. A further advantage of the invention includes producing the steel from thin continuously cast slabs. An additional advantage of the invention includes producing the steel using a reduced annealing temperature thereby effecting savings in annealing time and energy costs.

The above and other objects, features, and advantages of the invention will become apparent upon consideration of the detailed description.

### BRIEF DESCRIPTION OF THE DRAWINGS

FIG. 1 is a photomicrograph at 100x magnification of the grain structure of a cold reduced, recrystallization batch annealed steel for one embodiment of the invention,
FIG. 2 is a photomicrograph at 100x magnification of the grain structure of a steel having the same composition as that of FIG. 1 but having a grain structure outside the invention,
FIG. 3 is a photomicrograph at 100x magnification of the grain structure of a steel produced using the process of the invention but having an rₘ value outside the invention,
FIG. 4 is a photomicrograph at 100x magnification of the grain structure of a cold reduced, recrystallization batch annealed, aluminum killed steel having conventional composition and produced from a slab hot rolled from a conventional temperature,
FIG. 5 is a graph of the rₘ values of cold reduced, batch annealed, aluminum killed steel as a function of manganese composition for different slab temperatures and different hot rolling coiling temperatures,
FIG. 6 is a graph of the rₘ values of cold reduced, batch annealed, aluminum killed steel as a function of slab temperature for different acid sol. aluminum, total nitrogen and manganese compositions,
FIG. 7 is a graph of the rₘ values of cold reduced, aluminum killed steel as a function of batch annealing temperature, slab reheat temperature and manganese composition,
FIG. 8 is a graph of tensile strength for the steels of FIG. 7 as a function of batch annealing temperature, slab reheat temperature and manganese composition,
FIG. 9 is a graph of total elongation for the steels of FIG. 7 as a function of batch annealing temperature, slab reheat temperature and manganese composition,
FIG. 10 is a graph of the rₘ values of cold reduced, batch annealed, aluminum killed steels as a function of hot rolling time for different acid sol. aluminum, total nitrogen and manganese compositions,
FIG. 11 is a graph of the rₘ values as a function of the product of acid sol. aluminum and total nitrogen for cold reduced, aluminum killed steel hot rolled from a slab having a temperature of 1149°C at two different hot rolling times and batch annealed at 649°C for four hours,
FIG. 12 is a graph for rₘ values of cold reduced, aluminum killed steel as a function of batch annealing temperature for different acid sol. aluminum, total nitrogen and manganese compositions when hot rolled from a slab having a temperature of 1149°C,
FIG. 13 is a graph for rₘ values of cold reduced, aluminum killed steel as a function of aluminum nitrogen product, manganese and hot rolling time for steels hot rolled from a slab having a temperature of about 1149°C and annealed at 649°C - 4 hours.

### DETAILED DESCRIPTION OF THE PREFERRED EMBODIMENT

It will be understood by sheet is meant to include both cold reduced strip of indefinite length and cold reduced strip cut into definite lengths. It also will be understood the cold reduced sheets of the invention can be produced from slabs continuously cast from a melt or from ingots rolled on a slabbing mill.

The chemical composition of the steel in accordance with the present invention consists of ≤ 0.08% carbon, < 0.1% acid sol. aluminum ≤ 0.2% manganese, all percentages by weight and the balance of the composition being iron and unavoidable impurities.

As discussed in more detail below, the compositions of aluminum, nitrogen and manganese individually are important for flexibility in processing and good drawability. An equally important consideration is the product of aluminum and nitrogen, i.e., % acid sol. aluminum x % total nitrogen. I have determined the compositions for aluminum and nitrogen be controlled so that their product preferably is no greater than 5 x 10⁻⁴ and most preferably be within the range of 2 x 10⁻⁴ to 4 x 10⁻⁴. It is very important to control the aluminum nitrogen product when relatively long hot rolling times are required.

Manganese should be at least 0.05 wt.% to prevent hot shortness due to sulfur during hot rolling. If manganese is not low and exceeds about 0.24 wt.%, insufficient nitrogen would be retained in solution in hot rolled sheet produced from slabs having the reduced temperatures of the invention. To minimize slab and batch annealing temperatures and to maximize rₘ values, manganese preferably should be < 0.20 wt.% and most preferably ≤ 0.16 wt.%.

For an aluminum killed steel, at least 0.01 wt.% acid sol. aluminum is required to deoxidize the melt with the ratio of acid sol. aluminum to total nitrogen being at least 2:1. Maintaining this ratio insures that residual nitrogen exists as aluminum nitride so that recrystallization batch annealed steel is non-aging. For this reason, the acid sol. aluminum preferably should be at least 0.02 wt.%. Acid sol. aluminum should not exceed 0.1 wt.% because the annealed steel would have excessive hardness, diminished drawability and excess alloy cost. To minimize slab and batch annealing temperatures, to increase the elapsed times possible for hot rolling and to maximize rₘ values, acid sol. aluminum should be ≤ 0.08 wt.%. More preferably, acid sol. aluminum should be 0.03-0.08 wt.% and most preferably should be 0.05-0.06 wt.%.

Conventional residual amounts, i.e., impurities, of < 0.01 wt.% total nitrogen, < 0.02 wt.% phosphorus and < 0.018 wt.% sulfur are acceptable. To maximize drawability, total nitrogen preferably should be < 0.008 wt.%. More preferably, total nitrogen should be 0.003-0.007 wt.% and most preferably should be ≤ 0.004-0.006 wt.%.

Carbon should not exceed 0.08 wt.% because the batch annealed steel would have excessive hardness. Preferably, carbon is 0.03-0.05 wt.%.

Slabs of conventional thickness of 150-250 mm are hot rolled by gradually being reduced in thickness to about 30 mm by a series of roughing stands and further reduced to a sheet having a thickness of about 2.5 mm in a series of finishing stands. The hot rolled sheet then is coiled, descaled, cold reduced, and recrystallization batch annealed. Non-aging, aluminum killed steel produced by batch annealing requires nitrogen be retained in solid solution (not precipitated as aluminum nitride) in the hot rolled sheet after hot rolling.

Aluminum nitride precipitation during the heating stage of a batch annealing cycle results in the formation of the desired strong {111} recrystallization texture which provides rₘ values required for good drawing performance. For steel cold reduced and recrystallization batch annealed, thermal-mechanical processing of slabs during hot rolling is conducted in a manner so as to minimize the amount of aluminum nitride in the hot rolled sheet. In a paper entitled SOLUTION AND PRECIPITATION OF ALUMINUM NITRIDE IN RELATION TO THE STRUCTURE OF LOW CARBON STEELS, Trans. ASM, 46 (1954), p. 1470-1499, by W. C. Leslie et al, incorporated herein by reference, it is disclosed the solution temperature of aluminum nitride during hot rolling is a function of the product of the weight percentages of acid soluble aluminum and total nitrogen present in the steel. Whether continuously cast or produced from ingots, slabs of conventional thickness that have cooled to below the Ar₃ are reheated prior to hot rolling to a temperature of at least 1260°C for complete resolution of the aluminum nitride formed during cooling of the slab after casting. Following reheating, thick slabs are hot rolled through the roughing stands where the temperature of the slabs falls from about 1260°C to about 1040°C over a period of about 3.25 to 3.75 minutes. The steel at about 1040°C and having a thickness of 25-30 mm is further reduced to a thickness of about 2.5 mm by passing through a multi-stand finishing mill. The steel temperature falls from about 1040°C to a sheet exit temperature (finishing temperature) as low as about 870°C over a period of about 10 sec. Slabs preferably are processed to have a finishing temperature of at least 870°C to not only avoid aluminum nitride precipitation but also control grain size. Coiling temperature also is controlled to minimize aluminum nitride precipitation. On exiting the finishing mill, the sheet is water quenched to a temperature less than 650°C, more preferably to less than 593°C, and most preferably to 566°C before being wrapped into a coil. This is a suitable temperature from which to initiate the long time process of cooling the hot rolled sheet in coiled form and still avoid the precipitation of an undue amount of aluminum nitride. Thus, much of the nitrogen is retained in solution in the hot rolled sheet prior to cold reduction. Elevated coiling temperatures above 700°C result in excessive aluminum nitride precipitation virtually guaranteeing failure to obtain high rₘ values and good deep drawing properties following cold reduction and batch annealing.

I have determined slabs do not have to be reheated to a high temperature of 1260°C or more for hot rolling to obtain high rₘ values after batch annealing if manganese is lowered and aluminum and nitrogen is controlled. Slabs preferably are reheated to and hot rolled from a temperature less than 1175°C and most preferably from about 1149°C.

By way of example, aluminum killed steels were prepared in the laboratory by vacuum melting. Steels A-E were cast into slab ingots 28.6 mm thick, 102 mm wide, and 178 mm long and cooled to ambient. Four slabs for each steel composition were reheated from ambient temperature to 1093°C, 1149°C, 1204°C, and 1260°C for hot rolling. The residence time of the slabs in the heating furnace was one hour. The slabs were hot rolled to sheets having a thickness of 3.6 mm in about 0.5 minute, had a finishing temperature of 927°C, were water cooled to 566°C to simulate a coiling temperature and then slowly furnace cooled to ambient. The hot rolled sheets then were descaled by pickling and cold reduced 70% to a thickness of 1.07 mm. The cold reduced sheets were heated at a rate of 28°C/hr (simulating batch annealing) to a temperature of 649°C, were soaked at this temperature for 4 hours and then cooled at a rate of 28°C/hr. The annealed sheets were temper rolled 1%. The compositions by weight percent and rₘ values of the temper rolled sheets for steels A-E are shown in Table 1.

The results of Table 1 show that the steels for all manganese compositions had rₘ values of at least about 1.8 when using a conventional slab temperature of 1260°C. Steels A-D having manganese compositions less than 0.22 wt.% had very high rₘ values when the slabs were reheated to the reduced temperatures of 1149°C and 1204°C. In fact, using a slab temperature of only 1149°C resulted in exceptionally high rₘ values of 2.30 or more for steels A-D. However, further reducing the slab temperature to 1093°C resulted in very low rₘ values of 1.32 or less for all manganese compositions indicative apparently of insufficient nitrogen being retained in solution in the hot rolled sheet prior to cold reduction. Steel E had rₘ values less than 1.8 when hot rolled from slabs having reduced temperatures of 1149°C and 1204°C. Apparently, reducing the manganese content to 0.16 wt.% or less from 0.22 wt.% has a dramatic effect on the amount of nitrogen retained in solution in a hot rolled sheet rolled from a slab having a reduced temperature. By controlling the manganese content, apparently sufficient nitrogen was present in the hot rolled sheet for the formation of the recrystallization texture necessary for good rₘ values after batch annealing.

It is well known non-aging, cold reduced, batch annealed, aluminum killed steel is characterized by a grain structure having an elongation of 2.0 or more. Such a grain elongation is indicative that aluminum nitride precipitated during the slow heatup prior to the onset of recrystallization during annealing. It also is known the solution temperature of aluminum nitride is a function of the product of the weight percentages of nitrogen and aluminum in the steel. According to Leslie et al, the nitrogen and aluminum compositions of steels A-D would have suggested aluminum nitride "apparent" solution temperatures prior

**Table 1**

| | | | | | | CRBA rₘ Values* | | | |
|---|---|---|---|---|---|---|---|---|---|
| STEEL | C | N | Al(acid sol) | S | Mn | 1093°C | 1149°C | 1204°C | 1260°C |
| A | 0.046 | 0.007 | 0.07 | 0.008 | 0.07 | 1.32 | 2.48 | 2.26 | 1.78 |
| B | 0.044 | 0.007 | 0.07 | 0.007 | 0.10 | 1.26 | 2.38 | 1.91 | 2.45 |
| C | 0.036 | 0.008 | 0.07 | 0.008 | 0.13 | 1.21 | 2.39 | 1.89 | 1.94 |
| D | 0.046 | 0.007 | 0.07 | 0.008 | 0.16 | 1.19 | 2.30 | 1.93 | 1.89 |
| E | 0.042 | 0.007 | 0.08 | 0.009 | 0.22 | 1.09 | 1.44 | 1.71 | 1.79 |

| | | | | | | | | | |
|---|---|---|---|---|---|---|---|---|---|
| *rₘ Values For C R Steels BA At 649°C-4 Hours For Indicated Slab Reheat Temperatures And A Hot Rolling Coiling Temperature Of 566°C | | | | | | | | | |

**Table 2**

| | CRBArₘValues* | | | |
|---|---|---|---|---|
| STEEL | 1093°C | 1149°C | 1204°C | 1260°C |
| A | 1.30 | 1.28 | 1.41 | 1.35 |
| B | 1.21 | 1.26 | 1.30 | 1.29 |
| C | 1.21 | 1.28 | 1.25 | 1.27 |
| D | 1.13 | 1.21 | 1.21 | 1.21 |
| E | 1.11 | 1.15 | 1.13 | 1.15 |

| | | | | |
|---|---|---|---|---|
| * rₘ Values For C R Steels BA At 649°C-4 Hours For Indicated Slab Reheat Temperatures And A Hot Rolling Coiling Temperature Of 704°C | | | | |

to hot rolling of 1284°C or more. However, the grain structures of steels A-D after cold reduction and batch annealing had very high elongations well in excess of conventional elongations, i.e., ≥ 2.0, for reduced slab temperatures of 1149°C and 1204°C. For example, FIG. 1 shows a highly elongated grain structure for steel B having the rₘ value of 2.38 for the sheet that was cold reduced and batch annealed at 649°C for four hours. The sheet was produced from the slab reheated to 1149°C and having a simulated coiling temperature of 566°C after hot rolling. FIG. 2 shows an equiaxed grain structure for steel B having the rₘ value of 1.26 and having the same processing as steel B in FIG. 1 except the slab was reheated to 1093°C. FIG. 2 demonstrates a slab temperature of 1093°C apparently did not result in sufficient solute nitrogen in the hot rolled sheet to produce an elongated grain structure after cold reduction and batch annealing. FIG. 3 shows a conventional partially elongated grain structure for steel E having a low rₘ value of 1.44. Steel E in FIG. 3 had the same processing as steel B in FIG. 1 The only significant difference for steel E in FIG. 3 from that of steel B in FIG. 1 was that the steel in FIG. 3 had 0.22 wt.% manganese versus 0.10 wt.% for the steel in FIG. 1. It should be noted that not only was the elongation of the grain structure of the steel in FIG. 3 significantly less than that of the steel in FIG. 1 but also the grain structure of FIG. 3 includes a significant number of equiaxed grains. FIG. 4 shows a conventional elongated grain structure for steel E having the rₘ value of 1.79. Steel E in FIG. 4 was processed identically to steel B in FIG.1 except the slab was reheated to 1260°C. The grain structure of the steel in FIG. 4 having a conventional hot rolling slab temperature had a grain elongation approaching that of the steel in FIG. 1. Unlike the grain structure for steel E in FIG. 3 using a reduced hot rolling temperature, the grain structure for steel E in FIG. 4 using the conventional slab hot rolling temperature had very few equiaxed grains. The remaining steels A, C and D having reduced slab temperatures of 1149°C and 1204°C had similar grain elongations to that shown in FIG. 1. Steels A, C and D having a reduced slab temperature of 1093°C had grain structures similar to that shown in FIG. 2. Steels A, C and D having a conventional slab temperature of 1260°C had grain elongations similar to that shown in FIG. 1. Leslie et al teach steels A-D should not have had sufficient solute nitrogen in sheets hot rolled from slabs at the reduced temperatures of 1149°C and 1204°C, particularly 1149°C, to produce an elongated grain structure and high rₘ values after cold reduction and batch annealing. Contrary to these teachings, I determined that cold reduced and batch annealed steels A-D having manganese less than 0.22 wt.% and produced from sheets hot rolled from slabs reheated to temperatures of only 1149°C and 1204°C had grain elongations well in excess of conventional elongations. The reason for obtaining these elongated grain structures at reduced slab reheat temperatures is not known. Although not demonstrated analytically, a possible explanation for this unexpected result for steels A-D is that they apparently did have sufficient nitrogen retained in solution in the hot rolled sheet to form the classic elongated grain (and exceptionally high rₘ values) after cold reduction and simulated batch annealing.

In another experiment, steels A-E were processed identically to that for the example above reported in Table 1 except steels A-E were given an elevated simulated coiling temperature of 704°C instead of 566°C. The rₘ values are shown in Table 2.

For all compositions and slab reheat temperatures, the rₘ values were diminished to 1.41 or less for these batch annealed sheets. This suggests the elevated simulated coiling temperature caused the nitrogen to be precipitated as aluminum nitride prior to cold reduction. Conversely, these results appear to confirm that aluminum nitride was in solution after hot rolling for steels A-D in Table 1 having the reduced slab temperatures of 1149°C and 1204°C.

The rₘ values in Tables 1 and 2 are graphically shown in FIG. 5. Upper curve 10 shows the low manganese steels A-D having rₘ values well above 1.8 when cold reduced and batch annealed from sheet produced from slabs hot rolled at the reduced temperature of 1149°C and having a coiling temperature of 566°C. The rₘ value for steel E having identical processing dropped to 1.44. When the slab temperature for steel E was increased to the conventional temperature of 1260°C, the rₘ value was increased to 1.79. When the slabs for steels A-E were heated to 1149°C but had the simulated coiling temperature increased to 704°C, the rₘ values dropped to 1.28 or less as shown in curve 12. When the slabs for steels A-E were reheated to 1093°C and had a coiling temperature of 566°C, all rₘ values were 1.30 or less as shown in bottom curve 14.

During additional experimental work, I determined slabs could be rolled from a temperature as low as 1093°C and obtain rₘ values at least 1.8 after batch annealing by carefully controlling manganese, total nitrogen and acid sol. aluminum. Additional aluminum killed steels F-I were melted, cast into slab ingots, hot rolled to sheets in about 0.5 minute, pickled, cold reduced, batch annealed and then temper rolled identically to that for steels A-E in the example above reported in Table 1. The compositions by weight percent and rₘ values for steels F-I are shown in Table 3.

The results of Table 3 show that lowering manganese, total nitrogen and acid sol. aluminum had the effect of further reducing the slab temperature necessary prior to hot rolling and further increasing the rₘ value after batch annealing. A comparison of steels F and G shows steel G had a higher rₘ value at every slab temperature than the corresponding rₘ value of steel F. Similarly,

**Table 3**

| | | | | | | CRBA rₘ Values* | | | |
|---|---|---|---|---|---|---|---|---|---|
| STEEL | C | N | Al(acid sol.) | S | Mn | 1093°C | 1149°C | 1204°C | 1260°C |
| F | 0.042 | 0.009 | 0.08 | 0.007 | 0.22 | 1.21 | 1.76 | 1.65 | 1.68 |
| G | 0.039 | 0.003 | 0.04 | 0.008 | 0.22 | 1.78 | 2.31 | 1.95 | 1.77 |
| H | 0.044 | 0.008 | 0.08 | 0.008 | 0.12 | 1.34 | 2.07 | 1.71 | 1.80 |
| I | 0.041 | 0.004 | 0.04 | 0.007 | 0.12 | 1.88 | 2.25 | 2.26 | 2.28 |

| | | | | | | | | | |
|---|---|---|---|---|---|---|---|---|---|
| *rₘ Values For Cold Reduced Steels Batch Annealed At 649°C-4 Hours For Indicated Slab Reheat Temperatures And A Hot Rolling Coiling Temperature Of 566°C | | | | | | | | | |

a comparison of steels H and I shows steel I had a higher rₘ value at every slab temperature than the corresponding rₘ value of steel H as well. This clearly demonstrates the beneficial effect of increasing the rₘ values when reducing total nitrogen from about 0.009 to as low as 0.003 wt.% and reducing acid sol. aluminum from about 0.08 to as low as 0.04 wt.%. A similar comparison can be made demonstrating the beneficial effect of increasing the rₘ values when reducing manganese. Every rₘ value for steel H was higher than the corresponding rₘ value for steel F at each slab temperature. For steels I and G, every rₘ value for steel I was higher than the corresponding rₘ value for steel G at each slab temperature except for 1149°C where the rₘ values were substantially the same. Finally, steel I having low compositions for each of acid sol. aluminum, total nitrogen and manganese had dramatically higher rₘ values at all slab temperatures (except 1149°C for steel G) than the corresponding rₘ values for steels F, G and H which had higher acid sol. aluminum and total nitrogen and/or manganese. Furthermore, steel I demonstrated the slab temperature could be decreased at least about 170°C (from 1260°C or more to 1093°C or less) without decreasing drawability of cold reduced, batch annealed sheet thereby reducing energy cost. Surprisingly, drawability of the steel sheet can be expected to improve substantially (higher rₘ values) as well with this decrease in cost.

The results from Table 3 are graphically shown in FIG. 6. Lower curve 16 for steel F had rₘ values generally below 1.8 for all temperatures. Curve 18 for steel H had an rₘ value above 1.8 for the reduced slab temperature of 1149°C. This demonstrates the beneficial effect of increasing the rₘ values and being able to decrease the required slab temperature when decreasing manganese from 0.22 wt.% to 0.12 wt.%. Curve 20 for steel G demonstrates the beneficial effect of increasing the rₘ values and being able to decrease the required slab temperature when decreasing acid sol. aluminum and total nitrogen. The rₘ value was at least 1.8 for a slab temperature as low as 1093°C. Finally, curve 22 for steel I had rₘ values as good as or better than any of the other three steel compositions demonstrating the beneficial effect of improving drawability and reducing energy costs during hot rolling when the composition of acid sol. aluminum, total nitrogen and manganese are carefully controlled. The optimum slab temperature was 1149°C. Unlike none of the results reported in Table 1, steels G and I having relatively low acid sol. aluminum and total nitrogen had rₘ values of about 1.8 or more even when the slabs were reheated to only 1093°C.

Values for rₘ also were evaluated as a function of annealing temperature. By way of further example, aluminum killed steels J-Q were prepared and their compositions by weight percent are shown in Table 4.

**Table 4**

| STEEL | C | N | AL(acid sol.) | S | MN |
|---|---|---|---|---|---|
| J | 0.042 | 0.008 | 0.07 | 0.009 | 0.12 |
| K | 0.043 | 0.009 | 0.07 | 0.009 | 0.12 |
| L | 0.044 | 0.009 | 0.07 | 0.009 | 0.12 |
| M | 0.042 | 0.009 | 0.07 | 0.009 | 0.12 |
| N | 0.038 | 0.009 | 0.07 | 0.007 | 0.22 |
| O | 0.039 | 0.008 | 0.07 | 0.007 | 0.22 |
| P | 0.038 | 0.009 | 0.07 | 0.008 | 0.22 |
| Q | 0.038 | 0.009 | 0.07 | 0.007 | 0.22 |

Steels J-Q were cast into slab ingots, hot rolled to sheets, pickled, cold reduced, annealed and then temper rolled identically to that for steels A-E in the example above reported in Table 1. The slabs having hot rolling temperatures of 1149°C were hot rolled in about 0.5 minute and the slabs having hot rolling temperatures of 1260°C were hot rolled in 0.7 minute. Batch annealing temperatures of 566-732°C with a soak time of four hours were used. The rₘ values, yield strength, tensile strength and % total elongation after temper rolling are shown in Table 5 and graphically illustrated in FIGS. 7-9.

Curve 30 in FIG. 7 for steels N and O having relatively high acid sol. aluminum, total nitrogen and manganese of 0.07, 0.008-0.009 and 0.22 wt.% respectively conformed to the teachings of Leslie et al that using slab temperatures less than 1260°C did not produce acceptable rₘ values for batch annealed, aluminum killed steel. Curve 28 for steels P and Q hot rolled with a conventional slab temperature of 1260°C illustrates conventional rₘ values, i.e., generally < 1.8, for batch annealed, aluminum killed steel. Curve 26 for steels L and M hot rolled with a conventional slab temperature of 1260°C had improved rₘ values demonstrating the beneficial effect of very low manganese of .12 wt.%. Curve 24 for steels J and K had good rₘ values, i.e., ≥ 2.0, when hot rolled with a reduced slab temperature of 1149°C. Even more surprising was that the rₘ values for steels J and K hot rolled with a lower slab temperature were substantially higher than the rₘ values for steels L and M of the same composition but hot rolled from 1260°C. Aluminum killed steels having conventional manganese compositions and hot rolled from slab temperatures of 1260°C or more generally require batch annealing temperatures in excess of 649°C to develop conventional rₘ values and mechanical properties. Equally surprising was that steels J and K also had good rₘ values for an annealing temperature as low as 566°C. In addition to improving drawability and reducing energy costs during hot rolling, the invention can save energy cost and time during batch annealing as well.

**Table 5**

| STEEL | Slab Temp(°C) | Anneal Temp (°C) Time (hr) | rₘ Value | 0.2% Y.S. (N/mm²) | T.S. (N/mm²) | %Elong. |
|---|---|---|---|---|---|---|
| J | 1149 | 566-4 | 1.97 | 20.9 · 9.81 | 30.8 · 9.81 | 43.8 |
| J | 1149 | 593-4 | 2.34 | 20.7 · 9.81 | 30.2 · 9.81 | 43.8 |
| J | 1149 | 621-4 | 2.26 | 19.8 · 9.81 | 29.5 · 9.81 | 45.3 |
| J | 1149 | 649-4 | 2.41 | 17.9 · 9.81 | 28.8 · 9.81 | 48.5 |
| K | 1149 | 677-4 | 2.37 | 17.6 · 9.81 | 27.8 · 9.81 | 50.0 |
| K | 1149 | 704-4 | 2.42 | 16.6 · 9.81 | 26.9 · 9.81 | 48.0 |
| K | 1149 | 732-4 | 2.40 | 16.9 · 9.81 | 26.8 · 9.81 | 47.8 |
| L | 1260 | 566-4 | 1.76 | 23.6 · 9.81 | 35.2 · 9.81 | 31.5 |
| L | 1260 | 593-4 | 1.73 | 22.9 · 9.81 | 34.0 · 9.81 | 36.5 |
| L | 1260 | 621-4 | 1.94 | 18.2 · 9.81 | 30.6 · 9.81 | 42.3 |
| M | 1260 | 649-4 | 1.87 | 19.8 · 9.81 | 31.6 · 9.81 | 39.0 |
| M | 1260 | 677-4 | 2.01 | 19.7 · 9.81 | 31.2 · 9.81 | 41.8 |
| M | 1260 | 704-4 | 2.15 | 17.3 · 9.81 | 29.0 · 9.81 | 41.8 |
| M | 1260 | 732-4 | 2.01 | 18.3 · 9.81 | 29.3 · 9.81 | 45.0 |
| N | 1149 | 566-4 | 1.52 | 18.4 · 9.81 | 30.9 · 9.81 | 38.0 |
| N | 1149 | 593-4 | 1.38 | 20.7 · 9.81 | 30.7 · 9.81 | 41.0 |
| N | 1149 | 621-4 | 1.32 | 19.7 · 9.81 | 30.5 · 9.81 | 44.3 |
| N | 1149 | 649-4 | 1.41 | 18.2 · 9.81 | 29.7 · 9.81 | 46.3 |
| O | 1149 | 677-4 | 1.44 | 16.5 · 9.81 | 28.8 · 9.81 | 48.5 |
| O | 1149 | 704-4 | 1.64 | 17.0 · 9.81 | 27.9 · 9.81 | 44.5 |
| O | 1149 | 732-4 | 1.72 | 19.1 · 9.81 | 28.0 · 9.81 | 41.8 |
| P | 1260 | 566-4 | 1.47 | 27.2 · 9.81 | 37.2 · 9.81 | 34.0 |
| P | 1260 | 593-4 | 1.63 | 24.8 · 9.81 | 35.7 · 9.81 | 33.0 |
| P | 1260 | 621-4 | 1.59 | 23.6 · 9.81 | 34.2 · 9.81 | 38.5 |
| Q | 1260 | 649-4 | 1.68 | 22.9 · 9.81 | 33.0 · 9.81 | 41.5 |
| Q | 1260 | 677-4 | 1.73 | 18.0 · 9.81 | 31.0 · 9.81 | 43.0 |
| Q | 1260 | 704-4 | 1.56 | 19.1 · 9.81 | 29.9 · 9.81 | 42.5 |
| Q | 1260 | 732-4 | 1.79 | 17.9 · 9.81 | 29.3 · 9.81 | 49.8 |

Preferred tensile strength for deep drawing steel is no greater than about 313.9N/mm² (32 kg/mm²) with about 284.5-313.9N/mm² (29-32 kg/mm²) being the most preferred. Curves 32 and 34 in FIG. 8 are for steels J,K and N,O respectively having the reduced slab temperature of 1149°C. The annealing temperature preferably should be less than about 650°C to obtain the desired tensile strength. In contrast, curves 36 and 38 for steels L,M and P,Q respectively having the conventional slab temperature of 1260°C had increased tensile strengths at all annealing temperatures compared to those steels hot rolled from the slab temperature of 1149°C. Curves 32 and 34 illustrate that batch annealing temperature can be reduced for steels hot rolled from reduced slab temperatures.

Curves 40 and 42 in FIG. 9 correspond to steels J,K and N,O respectively and illustrate % total elongation as a function of batch annealing temperature. Curve 40 for steels J and K having very low manganese of .12 wt.% rolled from 1149°C had excellent total elongations at all annealing temperatures while curve 42 for steels N and O having 0.22 wt.% Mn also rolled from 1149°C had good total elongations at annealing temperatures of 600°C or more. Curves 44 and 46 correspond to steels L,M and P,Q respectively rolled from 1260°C. Steels L,M and P,Q had poor total elongations at annealing temperatures less than 650°C.

In the laboratory experiments referred to above, the total hot rolling time was a short 0.5 minute for steels having reduced slab temperatures. By total hot rolling time is meant the elapsed time necessary for rolling a slab through any roughing stands present in a hot rolling mill and rolling through the finishing stands. Conventional hot strip mills generally require long rolling times of about four minutes or more for slabs having thicknesses of 200 mm or more. In another experiment, rₘ values were determined as a function of total hot rolling time and aluminum and nitrogen content. Steels R-BB were cast into slab ingots, hot rolled to sheets, pickled, cold reduced, batch annealed and then temper rolled in a manner identical to that for the example above reported in Table 1 except hot rolling times of about 0.5, 2 and 4 minutes were used. The slab ingots were reheated from ambient in a furnace to 1149°C and held for one hour and then hot rolled to sheets having a thickness of 3.6 mm in three rolling passes. Steels hot rolled in 0.5 minute were held after the second pass until the temperature dropped to 949-943°C before completing the third pass. The finishing temperature after the third pass was 904°C. The steels immediately were water cooled and then slowly furnace cooled from 566°C to ambient. Steels hot rolled in about 2 minutes were processed similar to the previous procedure except the steels were held for 80 seconds in a furnace maintained at 982°C after the second pass. Steels rolled in about 4 minutes were hot rolled similar to the previous procedure except the steels were held for 200 seconds in the furnace maintained at 982°C after the second pass. Compositions by weight percent, the aluminum nitrogen product and the calculated fraction of aluminum nitride dissolved in the slabs at the reheat temperature of 1149°C, and mechanical properties for steels R-BB are shown in Table 6. Aluminum and nitrogen compositions having three and four significant digits respectively were used for calculating the aluminum nitrogen products and fraction of aluminum nitride dissolved at 1149°C even though aluminum and nitrogen compositions having only two and three significant digits respectively are reported in the tables herein. The rₘ values, tensile strength (TS) and total elongations (%Elong.) are for the steels after cold rolling 70%, batch annealing and temper rolling.

FIG. 10 graphically illustrates rₘ values as a function of hot rolling times for steels R-Z and BB hot rolled from slabs reheated to 1149°C and batch annealed at 649°C for four hours. A curve for steel AA was excluded from FIG. 10 since the rₘ values were essentially the same as those for steel BB. Curve 46 for steel R having relatively high concentrations for nitrogen, aluminum and manganese had low rₘ values for hot rolling times of two minutes or more. Curve 48 for steel S had a composition similar to steel R except steel S had very low manganese. Steel S had improved rₘ values at all hot rolling times but the rₘ values still were unacceptable at times of two minutes or more. Curve 50 for steel T had a composition similar to steel S except nitrogen was substantially reduced. Steel T had greatly improved rₘ values at all hot rolling times and were about 2.0 at times of two minutes or more. Curve 52 for steel U had a composition and rₘ values similar to steel T at hot rolling times of 0.5 and 2 minutes. Remaining steels V-Z and BB (curves 54-64 respectively) had low aluminum, nitrogen and manganese except steel Y had 0.23 wt.% manganese and steel Z had 0.07 wt.% acid sol. aluminum. Steels V-Z and BB had good rₘ values at all hot rolling times. Steel Y (curve 60) having 0.23 wt.% manganese had acceptable rₘ values at all hot rolling times and an rₘ value of about 2.0 for hot rolling times of 0.5 and 4 minutes. Curves 62 and 64 for steels Z and BB respectively having total nitrogen of 0.003 wt.% had acceptable rₘ values of about 1.9 or more at all rolling times. Surprisingly, steels Z and BB had the highest calculated fraction of aluminum nitride (100%) dissolved in the hot rolled sheet but did not have the highest rₘ values. Steels T, U, V and W had rₘ values higher than the rₘ values for steels Z and BB at all hot rolling times even though steels T, U, V and W had only about 40%, 49%, 56% and 67% respectively of aluminum nitride apparently dissolved at the 1149°C reheat temperature prior to hot rolling. Steels T, U, V and W should have had more than 0.002 wt.% nitrogen retained in solution after hot rolling. This demonstrates for batch annealed, aluminum killed steel having low manganese that aluminum nitride need not be completely dissolved during slab reheating prior to hot rolling. The absolute amount of nitrogen retained in solution following hot rolling appears more important than the fraction retained. For optimum rₘ values, Table 6 and FIG. 10 demonstrate total nitrogen preferably should be 0.004-0.006 wt.% with at least about 0.002 wt.% nitrogen retained in solution following hot rolling.

As graphically demonstrated in FIG. 10, rₘ values for batch annealed, aluminum killed steels appear to be a function not only of nitrogen, aluminum and manganese but also total time for hot rolling as well. It appears important to control aluminum and nitrogen, even when manganese was controlled to less than 0.20 wt.%, when relatively long hot rolling times of two minutes or more are required when using slab temperatures less than 1260°C to obtain rₘ values of at least about 1.8 after batch annealing. When hot rolling times are two minutes or more and manganese was controlled to ≤ 0.16 wt.%, acid sol. aluminum can be as high as 0.08 wt.% with total nitrogen as high as 0.007 wt.% provided the product of % acid sol. aluminum and % total nitrogen was no greater than about 5 x 10⁻⁴. When hot rolling times are two minutes or more and acid sol. aluminum and total nitrogen are controlled to no more than about 0.05 and 0.005 wt.% respectively, manganese can be at least 0.23 wt.%.

The relationship between aluminum and nitrogen to rₘ values also can be expressed as a function of the aluminum nitrogen product, i.e., wt.% acid sol. Al x wt.% total N. Steels C, H, I, J, S, T, U, V, W, X, Z, AA and BB all had low manganese of 0.11-0.13 wt.%. Two samples of each of these steels, except steels C, H, I and J, were hot rolled at times of about 0.5 and 2 minutes and batch annealed at 649°C for four hours. Steels C, H, I and J were hot rolled only at a time of about 0.5 minute. The rₘ values as a function of the aluminum nitrogen product are illustrated in FIG. 11. For both hot rolling times, the rₘ values increased with increasing aluminum nitrogen product with optimum rₘ values obtained at about an aluminum nitrogen product of about 3 x 10⁻⁴. With a further increase in the aluminum nitrogen product, rₘ values decreased as illustrated by curve 66 for a rolling time of 0.5 minute and curve 68 for a rolling time of 2 minutes. The results for a rolling time of 4 minutes were substantially the same as for the 2 minute rolling time (see Table 6). Low manganese steels having a short hot rolling time of 0.5 minute had acceptable rₘ values for all aluminum nitrogen product values. For longer hot rolling times of 2 minutes, however, acceptable rₘ values of 1.8 or more were obtained so long as the aluminum nitrogen product did not exceed about 5 x 10⁻⁴. For example, for steels having 0.11-0.13 wt.% manganese and having 0.08 wt.% acid sol. aluminum, total nitrogen should not exceed about 0.006 wt.%. Interestingly, the left hand portions of curves 66 and 68 both suggest the aluminum nitrogen product should not be less than about 1 x 10⁻⁴. That is, for steels having 0.03 wt.% acid sol. aluminum, total nitrogen should be at least 0.004 wt.%. Alternatively, for steels having 0.003 wt.% or less total nitrogen, acid sol. aluminum should be at least 0.04 wt.%. In any case, total nitrogen should not be less than 0.003 wt.%. Otherwise, insufficient solute nitrogen would be available after hot rolling at the hot band stage to precipitate during heating in batch annealing following cold rolling. For optimum rₘ values, aluminum nitrogen product should be 2 x 10⁻⁴ to 4 x 10⁻⁴.

Steels R-BB hot rolled for four minutes from slabs reheated to 1149°C were batch annealed at temperatures of 649°C, 607°C and 566°C. Steels V, W and X also were batch annealed at 538°C. The rₘ values as a function of annealing temperature for steels R, V, X and Y are illustrated in FIG. 12. It does not appear steel R (curve 70) having relatively high concentrations for nitrogen, aluminum and manganese will develop good rₘ values at any annealing temperature when a long hot rolling time of four minutes is required. Steel Y (curve 72) having low nitrogen and aluminum but relatively high manganese of 0.23 wt.% developed good rₘ values at annealing temperatures of about 600°C and higher for the four minute rolling time. Steels V and X (curves 74 and 76 respectively) having low nitrogen, aluminum and manganese developed excellent rₘ values at all annealing temperatures. Steels V and X surprisingly had excellent rₘ values at an annealing temperature of only 566°C for the four minute rolling time. Steels V, W and X also were batch annealed at 538°C for 8 hours instead of 4 hours. Steels V, W and X had acceptable rₘ values when batch annealed at 538°C with steels V and X still having excellent rₘ values and mechanical properties. Steel W was not quite fully recrystallized after batch annealing at 538°C. While it had a good rm value of 1.8, the tensile properties of steel W were unaceptable.

To more clearly illustrate the interdependence between manganese, aluminum nitrogen product and hot rolling time for slabs rolled from temperatures less than 1260°C, the results of several of the steels described above are recast in Table 7. Table 7 shows the rₘ values following batch annealing at 649°C - 4 hours for those steels having either 0.12-0.13 or 0.22-0.23 wt. % manganese, aluminum nitrogen products in the range of about 1.4 x 10⁻⁴ to 7.5 x 10⁻⁴, hot rolled from a slab having a temperature of about 1149°C and having a hot rolling time of either 0.5 or 2 minute. Table 7 was constructed by grouping steels at the two manganese compositions according to values of aluminum nitrogen product as close as possible to one another over the above cited range. The results are graphically illustrated in FIG. 13. Curve 78

**TABLE 7**

| Steel | Mn | Al (acid sol.) | N(total) | [%Al][%N] x 10,000 | H. R.Time 0.5 min. rₘ Value* | H. R.Time 2 min. rₘ Value* |
|---|---|---|---|---|---|---|
| S | 0.12 | 0.07 | 0.009 | 6.25 | 2.20 | -- |
| N | 0.22 | 0.07 | 0.009 | 6.32 | 1.41 | -- |
| T | 0.13 | 0.08 | 0.006 | 5.25 | 2.43 | -- |
| T | 0.13 | 0.08 | 0.006 | 5.17 | -- | 2.01 |
| U | 0.13 | 0.07 | 0.007 | 4.23 | 2.57 | -- |
| U | 0.13 | 0.07 | 0.007 | 4.36 | -- | 2.05 |
| X | 0.12 | 0.05 | 0.004 | 2.13 | 2.51 | -- |
| Y | 0.23 | 0.05 | 0.004 | 2.17 | 1.98 | -- |
| I | 0.12 | 0.04 | 0.004 | 1.37 | 2.25 | -- |
| G | 0.22 | 0.04 | 0.003 | 1.47 | 2.31 | -- |
| S | 0.12 | 0.07 | 0.009 | 6.67 | -- | 1.46 |
| R | 0.22 | 0.09 | 0.009 | 7.48 | -- | 1.27 |
| X | 0.12 | 0.05 | 0.004 | 2.23 | -- | 2.47 |
| Y | 0.23 | 0.05 | 0.004 | 2.23 | -- | 1.90 |

| | | | | | | |
|---|---|---|---|---|---|---|
| * Hot Rolled From 1149°C And Batch Annealed 649°C - 4 Hours | | | | | | |

demonstrates for a short rolling time of 0.5 minute and low manganese of ≤ 0.13 wt.%, the rₘ values are very high, i.e., ≥ 2.0, for aluminum nitrogen products over the range 1.4 x 10⁻⁴ to 6.3 x 10⁻⁴. Curve 80 demonstrates for a relatively long rolling time of 2 minutes and low manganese of ≤ 0.13 wt.%, the rₘ values also are very high up to an aluminum nitrogen product of about 5 x 10⁻⁴. The rₘ value was substantially below 1.8 (steel S) when the aluminum nitrogen product exceeds about 5 x 10⁻⁴. Curve 82 demonstrates for a rolling time of about 0.5 minute and relatively high manganese of 0.22-0.23 wt.%, the rₘ value was very low, e.g., 1.4, for steel N when the aluminum nitrogen product increased to about 6.3 x 10⁻⁴. This was in direct contrast to steel S having the rolling time of about 0.5 minute, 0.12 wt.% Mn and a relatively high aluminum nitrogen product of about 6.3 x 10⁻⁴ illustrated by curve 78. Curve 82 also demonstrates for the rolling time of about 0.5 minute, steels Y and G having relatively high 0.22-0.23 wt.% Mn and a low aluminum nitrogen product of about ≤ 2.2 x 10⁻⁴, the rₘ values still were very high but somewhat lower than the rₘ values for steels X and I having 0.12 wt.% Mn and the same aluminum nitrogen product. Curve 82 further demonstrates for the rolling time of about 0.5 minute, regardless of the manganese composition when the aluminum nitrogen was about 1.4 x 10⁻⁴, the rₘ values are very high and essentially the same, e.g., 2.3. Comparing curve 84 for relatively high 0.22-0.23 wt.% Mn and the 2 minute rolling time to curve 82 for the same manganese but a 0.5 minute rolling time demonstrates there was little influence of rolling time on the rₘ values when the manganese was relatively high, i.e., ≥ 0.20 wt%. In contrast, comparing curve 80 for ≤ 0.13 wt.% Mn and the 2 minute rolling time to curve 78 having the same manganese and the 0.5 minute rolling time demonstrates there was a significant influence of rolling time on the rₘ values when the manganese was very low, i.e., < 0.20 wt.%. Even so, rₘ values were remarkably superior for

steels having ≤ 0.13 wt.% Mn versus 0.22-0.23 wt.% Mn for a 2 minute rolling time over an aluminum nitrogen product range of about 2 x 10⁻⁴ to 5 x 10⁻⁴.

All the features of the invention are demonstrated in a final experiment wherein rₘ values were determined for a steel CC having optimum aluminum and nitrogen content of 0.05 wt.% and 0.005 wt.% respectively, optimum aluminum nitrogen product of about 2.5 x 10⁻⁴, a conventional total hot rolling time of about four minutes and a low manganese composition of 0.11 wt.%. The rₘ values of steel CC are compared to the rₘ values of a steel DD having the same optimum composition except for relatively high manganese of 0.21 wt.%. Steels CC and DD were cast into slab ingots, hot rolled to sheets, pickled, cold reduced, batch annealed and then temper rolled in a manner identical to that for the example reported in Table 6 except only a hot rolling time of 4 minutes was used for slab reheat temperatures of 1149°C, 1204°C and 1260°C. Samples for each steel were batch annealed at temperatures of 649°C, 607°C and 566°C for four hours. The results are shown in Table 8 and demonstrate rₘ value was not adversely effected using reduced slab reheat temperature or reduced annealing temperature. In fact, rₘ values for the reduced slab reheat temperature of 1149°C generally equaled or exceeded the rₘ values for the conventional reheat temperature of 1260°C for steels CC and DD. For the reduced annealing temperature of 566°C, the rₘ values were slightly less than the rₘ values for the annealing temperature of 649°C. As demonstrated above in Table 7, there is a clear interdependence between manganese and rₘ values. The rₘ values of low manganese steel CC exceeded the rₘ values for relatively high manganese steel DD at all annealing temperatures. Nevertheless, even for relatively high manganese of .21 wt.%, the rₘ values were still good, i.e., at least 1.8, using a reduced slab reheat temperature of 1149°C and a reduced annealing temperature of 566°C when aluminum, nitrogen and the aluminum nitrogen product all were carefully controlled.

Those skilled in the art will appreciate slabs having conventional thicknesses of 150-250 mm need an initial temperature of 1200°C or more to be hot rolled to a thickness of about 2.5 mm and have a finishing temperature of at least 870°C. The most preferred slab temperature of the invention of no more than about 1149°C has practical application for thin continuously cast slabs having thicknesses of 25-50 mm. Additional cost savings are possible by casting a melt into thin slabs rather than thick slabs having a conventional thickness of 150 mm or more. By casting into a thin slab, time and energy for hot rolling to a sheet would be minimized. For example, a thin slab would require no or only minimal reduction using roughing stands. In addition to saving time and energy during rolling, further energy could be saved because the initial slab temperature could be considerably less than that required for thick slabs. Instead of at least 1260°C, thin slabs can be heated to as low as 1093°C and still be satisfactorily hot rolled into a non-aging, batch annealed, aluminum killed steel having very a high rₘ value.

The steel of the invention can be produced from continuously cast thin or thick slabs as well as thick slabs produced from ingots. Various reduced slab temperatures can be used so long as the hot rolling finishing temperature is above Ar₃ and the coiling temperature is below 593°C. The limits of the invention are determined from the appended claims.

## Claims

1. Method of producing an aluminum killed steel, comprising:
providing a slab comprising, by weight, 0.03 - 0.08 % carbon, ≤ 0.24 % manganese, ≥ 0.01 acid sol. % aluminum and nitrogen as an impurity, wherein the product of % acid sol. aluminum and % total nitrogen is no greater than 5 x 10⁻⁴, the balance being iron and unavoidable impurities,
cooling said slab to a temperature less than about Ar₃ to precipitate aluminum nitride,
reheating said slab to a temperature less than 1260 °C prior to said hot rolling to redissolve said aluminum nitride,
hot rolling said slab having a hot rolling temperature less than about 1260 °C to a sheet having nitrogen in solution,
coiling said hot rolled sheet at a temperature range of more than 500 °C to 593 °C,
descaling said hot rolled sheet,
cold reducing said descaled sheet,
recrystallization batch annealing without decarburization said cold reduced sheet, wherein said annealed sheet is non-aging, has an elongated grain structure and has an rₘ value of at least 1.8.

2. Method according to claim 1, characterized in that the batch annealing is at a temperature no greater than 649 °C.

3. Method according to claim 1, characterized in that said batch annealing is at a temperature of at least 538 °C.

4. Method according to one of the claims 1 to 3, characterized in that the slab has 0.03 - 0.08 % acid sol. aluminum and said rₘ value is at least 2.0.

5. Method according to anyone of the claims 1 to 4, characterized in that the slab has 0.003 - 0.007 % total nitrogen and said rₘ value is at least 2.0.

6. Method according to anyone of the claims 1 to 5, characterized in that the slab has < 0.20 % manganese and said rₘ value is at least 2.0.

7. Method according to anyone of the claims 1 to 6, characterized in that the slab has 0.05 - 0.06 % acid sol. aluminum, 0.004 - 0.006 % total nitrogen, the product of % acid sol. aluminum and % total nitrogen is in the range of 2 x 10⁻⁴ to 4 x 10⁻⁴ and said rₘ value is at least 2.0.

8. Method according to anyone of the claims 1 to 7, characterized in that the batch annealed sheet has a tensile strength of 284.5 - 313.9 N/mm² (29 - 32 kg/mm²) and a total elongation of at least 42 %.

9. Method according to anyone of the claims 1 to 8, characterized in that the slab is continuously cast to a thickness of about 25 - 50 mm.

10. Method according to claim 9, characterized in that
- a melt for casting the slab comprises ≤ 0.05 % carbon, ≤ 0.03 - 0.08 % acid sol. aluminum, 0.003 - 0.007 % total nitrogen, ≤ 0.24 % manganese, wherein the product of % acid sol. aluminum and % total nitrogen is no greater than 5 x 10⁻⁴, all percentages by weight, the balance being iron and unavoidable impurities,
- after cooling the cast slab to the temperature below Ar₃ the slab is reheated to a temperature less than 1175 °C to redissolve the aluminum nitride.

11. Method according to claim 10, characterized in that said melt comprises ≤ 0.05 % carbon, 0.05 - 0.06 % acid sol. aluminum, 0.004 - 0.006 % total nitrogen, ≤ 0.24 % manganese, wherein the product of % acid sol. aluminum and % total nitrogen is within the range of 2 x 10⁻⁴ to 4 x 10⁻⁴, all percentages by weight, the balance being iron and unavoidable impurities,
the step of hot rolling said slab to a sheet has a finishing temperature at least equal to Ar₃, and the step of recrystallization batch annealing without decarburization said cold reduced sheet is in the range of 538 - 649 °C.

12. Method according to claim 1, characterized in that a melt is provided, comprising 0.03 - 0.08 % carbon, ≤ 0.24 % manganese, ≥ 0.01 acid sol. % aluminum and nitrogen as an impurity wherein the product of % acid sol. aluminum and % total nitrogen is no greater than 5 x 10⁻⁴, all percentages by weight, the balance being iron and unavoidable impurities,
said melt is continuously cast to a slab having a thickness of 25 - 50 mm, said slab is cooled to a temperature below Ar₃ to precipitate aluminum nitride, said slab is reheated to a temperature less than 1175 °C to redissolve said aluminum nitride,
said slab is hot rolled to a sheet having nitrogen in solution, and
after coiling said hot rolled sheet, descaling said hot rolled sheet, cold reducing said descaled sheet, and recrystallization batch annealing without decarburization said cold reduced sheet, said annealed sheet is non-aging, has an elongated grain structure and has an rₘ value of at least 2.0.

## Patentansprüche

1. Verfahren zur Herstellung von aluminiumberuhigtem Stahl, das umfaßt:
Bereitstellen eines Flachguts mit 0,03 bis 0,08 Gew.% Kohlenstoff, ≤ 0,24 Gew.% Mangan, ≥ 0,01 Gew.% säurelöslichem Aluminium und Stickstoff als eine Verunreinigung, wobei das Produkt aus dem Prozentgehalt an säurelöslichem Aluminium und dem Prozentgehalt an Gesamtstickstoff nicht größer ist als 5 x 10⁻⁴ und der Restgehalt aus Eisen und unvermeidbaren Verunreinigungen besteht,
Abkühlen des Flachguts auf eine Temperatur kleiner als Ar₃ zur Ausscheidung von Aluminiumnitrid,
Wiedererhitzen des Flachguts auf eine Temperatur kleiner als 1260 °C vor dem Warmwalzen, um das Aluminiumnitrid wieder zu lösen,
Warmwalzen des eine Warmwalztemperatur von weniger als ungefähr 1260 °C aufweisenden Flachguts zu einem Stickstoff in Lösung enthaltenden Blech,
Aufwickeln des warmgewalzten Blechs in einem Temperaturbereich von größer als 500 bis 593 °C,
Entzundern des warmgewalzten Blechs,
Kaltreduzieren des entzunderten Blechs,
Rekristallisations-Chargenglühen ohne Entkohlung des kaltreduzierten Blechs, wobei das geglühte Blech alterungsbeständig ist und eine langgestreckte Kornstruktur und einen rₘ-Wert von wenigstens 1,8 aufweist.

2. Verfahren nach Anspruch 1, dadurch gekennzeichnet, daß das Chargenglühen bei einer Temperatur nicht höher als 649 °C stattfindet.

3. Verfahren nach Anspruch 1, dadurch gekennzeichnet, daß das Chargenglühen bei einer Temperatur von wenigstens 538 °C stattfindet.

4. Verfahren nach einem der Ansprüche 1 bis 3, dadurch gekennzeichnet, daß das Flachgut 0,03 bis 0,08 Gew.% an säurelöslichem Aluminium enthält und der rₘ-Wert wenigstens 2,0 beträgt.

5. Verfahren nach einem der vorstehenden Ansprüche 1 bis 4, dadurch gekennzeichnet, daß das Flachgut 0,003 bis 0,007 Gew.% Gesamtstickstoff enthält und der rₘ-Wert wenigstens 2,0 beträgt.

6. Verfahren nach einem der Ansprüche 1 bis 5, dadurch gekennzeichnet, daß das Flachgut < 0,20 Gew.% Mangan enthält und der rₘ-Wert wenigstens 2,0 beträgt.

7. Verfahren nach einem der vorstehenden Ansprüche 1 bis 6, dadurch gekennzeichnet, daß das Flachgut 0,05 bis 0,06 Gew.% säurelösliches Aluminium und 0,004 bis 0,006 Gew.% Gesamtstickstoff enthält und das Produkt aus dem Prozentgehalt an säurelöslichem Aluminium und dem Prozentgehalt an Gesamtstickstoff im Bereich von 2 x 10⁻⁴ bis 4 x 10⁻⁴ liegt und der rₘ-Wert wenigstens 2,0 beträgt.

8. Verfahren nach einem der vorstehenden Ansprüche 1 bis 7, dadurch gekennzeichnet, daß das chargengeglühte Blech eine Zugfestigkeit von 284,5 bis 313,9 N/mm² (29 bis 32 kg/mm²) und eine Gesamtdehnung von wenigstens 42 % aufweist.

9. Verfahren nach einem der Ansprüche 1 bis 8, dadurch gekennzeichnet, daß das Flachgut kontinuierlich bis zu einer Dicke von 25 bis 50 mm vergossen wird.

10. Verfahren nach Anspruch 9, dadurch gekennzeichnet, daß
- eine Schmelze zum Gießen des Flachguts ≤ 0,05 Gew.% Kohlenstoff, ≤ 0,03 bis 0,08 Gew.% säurelösliches Aluminium, 0,003 bis 0,007 Gew.% Gesamtstickstoff und ≤ 0,24 Gew.% Mangan enthält, wobei das Produkt aus dem Prozentgehalt an säurelöslichem Aluminium und dem Prozentgehalt an Gesamtstickstoff nicht größer ist als 5 x 10⁻⁴, und der Restgehalt aus Eisen und unvermeidbaren Verunreinigungen besteht,
- das Flachgut nach dem Abkühlen des gegossenen Flachguts auf eine Temperatur unterhalb Ar₃ wieder auf eine Temperatur kleiner als 1175 °C erhitzt wird, um das Aluminiumnitrid wieder zu lösen.

11. Verfahren nach Anspruch 10, dadurch gekennzeichnet, daß die Schmelze ≤ 0 05 Gew.% Kohlenstoff, 0,05 bis 0,06 Gew.% säurelösliches Aluminium, 0,004 bis 0,006 Gew.% Gesamtstickstoff und ≤ 0,24 Gew.% Mangan enthält, wobei das Produkt aus dem Prozentgehalt an säurelöslichem Aluminium und dem Prozentgehalt an Gesamtstickstoff innerhalb des Bereichs von 2 x 10⁻⁴ bis 4 x 10⁻⁴ liegt, der Restgehalt aus Eisen und unvermeidbaren Verunreinigungen besteht, der Schritt des Warmwalzens des Flachguts zu einem Blech eine Endbearbeitungstemperatur aufweist, die wenigstens gleich Ar₃ ist, und der Schritt des Rekristallisations-Chargenglühens ohne Entkohlung des kaltreduzierten Blechs im Bereich von 538 bis 649 °C stattfindet.

12. Verfahren nach Anspruch 1, dadurch gekennzeichnet, daß eine Schmelze bereitgestellt wird, die 0,03 bis 0,08 Gew.% Kohlenstoff, ≤ 0,24 Gew.% Mangan, ≥ 0 01 Gew.% säurelösliches Aluminium und Stickstoff als eine Verunreinigung aufweist, wobei das Produkt aus dem Prozentgehalt an säurelöslichem Aluminium und dem Prozentgehalt an Gesamtstickstoff nicht größer als 5 x 10⁻⁴ ist und der Restgehalt aus Eisen und unvermeidbaren Verunreinigungen besteht,
diese Schmelze kontinuierlich zu einem Flachgut mit einer Dicke von 25 bis 50 mm vergossen wird, das Flachgut auf eine Temperatur kleiner als Ar₃ abgekühlt wird, um Aluminiumnitrid auszuscheiden, das Flachgut wieder auf eine Temperatur kleiner als 1175 °C erhitzt wird, um das Aluminiumnitrid wieder zu lösen,
das Flachgut zu einem Blech warmgewalzt wird, das Stickstoff in Lösung aufweist, und
nach dem Aufwickeln des warmgewalzten Blechs Entzundern des warmgewalzten Blechs, Kaltreduzieren des entzunderten Blechs und Rekristallisations-Chargenglühen ohne Entkohlung des kaltreduzierten Blechs, das geglühte Blech ist alterungsbeständig und weist eine langgestreckte Kornstruktur und einen rₘ-Wert von wenigstens 2,0 auf.

## Revendications

1. Procédé de production d'acier calme à l'aluminium, comprenant :
l'utilisation d'une brame comprenant en poids 0,03 - 0,08 % de carbone, ≤ 0,24 % de manganèse, ≥ 0,01 % d'aluminium soluble dans l'acide et de l'azote en tant qu'impureté, le produit du pourcentage d'aluminium soluble dans l'acide et du pourcentage total d'azote n'étant pas supérieur à 5 x 10⁻⁴, le reste étant formé de fer et d'impuretés inévitables,
le refroidissement de ladite brame à une température inférieure à environ Ar₃ pour faire précipiter du nitrure d'aluminium,
le réchauffage de ladite brame à une température inférieure à 1260°C avant ledit laminage à chaud pour dissoudre à nouveau ledit nitrure d'aluminium,
le laminage à chaud de ladite brame s'effectuant à une température de laminage à chaud inférieure à environ 1260°C pour obtenir une feuille contenant de l'azote en solution, l'enroulement de ladite feuille laminée à chaud dans une gamme de températures allant de plus de 500°C à 593°C,
le décapage de ladite feuille laminée à chaud,
le formage à froid de ladite feuille décapée,
le recuit discontinu de recristallisation sans décarburation de ladite feuille réduite par formage à froid, ladite feuille ayant subi le recuit n'étant pas sujette au vieillissement, possédant une structure granulaire allongée et ayant une valeur Rₙ égale au moins à 1,8.

2. Procédé selon la revendication 1, caractérisé en ce que le recuit discontinu s'effectue à une température non supérieure à 649°C.

3. Procédé selon la revendication 1, caractérisé en ce que ledit recuit discontinu s'effectue à une température égale à au moins 538°C.

4. Procédé selon l'une des revendications 1 à 3, caractérisé en ce que la brame possède 0,03 - 0,08 % d'aluminium soluble dans l'acide et ladite valeur Rₘ est égale à au moins 2,0.

5. Procédé selon l'une quelconque des revendications 1 à 4, caractérisé en ce que la brame possède 0,003 - 0,007 % d'azote total et ladite valeur Rₘ est égale à au moins 2,0.

6. Procédé selon l'une quelconque des revendications 1 à 5, caractérisé en ce que la brame possède < 0,20 % de manganèse et ladite valeur Rₘ est égale à au moins 2,0.

7. Procédé selon l'une quelconque des revendications 1 à 6, caractérisé en ce que la brame possède 0,05 - 0,06 % d'aluminium soluble dans l'acide, 0,004 - 0,006 % d'azote total, le produit du pourcentage d'aluminium soluble dans l'acide par le pourcentage d'azote total est situé dans la gamme comprise entre 2 x 10⁻⁴ et 4 x 10⁻⁴, et ladite valeur Rₘ est égale à au moins 2,0.

8. Procédé selon l'une quelconque des revendications 1 à 7, caractérisé en ce que la feuille soumise à un recuit discontinu possède une résistance à la traction égale à 284,5 - 313,9 N/mm² (29 - 32 kg/mm²) et un allongement total égal à au moins 42 %.

9. Procédé selon l'une quelconque des revendications 1 à 8, caractérisé en ce que la brame est coulée en continu à une épaisseur d'environ 25 - 50 mm.

10. Procédé selon la revendication 9, caractérisé en ce que
- une masse fondue pour la coulée de la brame comprend ≤ 0,05 % de carbone, ≤ 0,03 - 0,08 % d'aluminium soluble dans l'acide, 0,003 - 0,007 % d'azote total, ≤ 0,24 % de manganèse, le produit du pourcentage d'aluminium soluble dans l'acide par le pourcentage d'azote total n'étant pas supérieur à 5 x 10⁻⁴, tous les pourcentages étant exprimés en poids, le reste étant constitué par du fer et par des impuretés inévitables,
- après refroidissement de la brame coulée à la température inférieure à Ar₃, on réchauffe la brame à une température inférieure à 1175°C pour effectuer une nouvelle dissolution du nitrure d'aluminium.

11. Procédé selon la revendication 10, caractérisé en ce que ladite masse fondue comprend ≤ 0,05 % de carbone, 0,05 - 0,06 % d'aluminium soluble dans l'acide, 0,004 - 0,006 % d'azote total, ≤ 0,24 % de manganèse, le produit du pourcentage d'aluminium soluble dans l'acide par le pourcentage d'azote total se situant dans la gamme comprise entre 2 x 10⁻⁴ et 4 x 10⁻⁴, tous les pourcentages étant indiqués en poids, le reste étant constitué de fer et d'impuretés inévitables,
l'étape de laminage à chaud de ladite brame pour former une feuille fait intervenir une température de finition au moins égale à Ar₃, et l'étape de recuit discontinu de recristallisation sans décarburation de ladite feuille réduite par formage à froid se situe dans la gamme de 538 - 649°C.

12. Procédé selon la revendication 1, caractérisé en ce qu'il est prévu une masse fondue, comprenant 0,03 - 0,08 % de carbone, ≤ 0,24 % de manganèse, ≥ 0,01 % d'aluminium soluble dans l'acide, et de l'azote en tant qu'impuretés, le produit du pourcentage d'aluminium soluble dans l'acide par le pourcentage d'azote total n'étant pas supérieur à 5 x 10⁻⁴, tous les pourcentages étant exprimés en poids, le reste étant formé de fer et d'impuretés inévitables,
ladite masse fondue est coulée en continu sous la forme d'une brame ayant une épaisseur de 25 - 50 mm, ladite brame est refroidie à une température inférieure à Ar₃ pour faire précipiter le nitrure d'aluminium, ladite brame est réchauffée à une température inférieure à 1175°C pour faire dissoudre à nouveau ledit nitrure d'aluminium,
ladite brame est laminée à chaud pour former une feuille comportant de l'azote en solution, et
après enroulement de ladite feuille laminée à chaud, décapage de ladite feuille laminée à chaud, formage à froid de ladite feuille décapée et recuit discontinu de recristallisation sans décarburation de ladite feuille réduite par formage à froid, ladite feuille ayant subi le recuit n'est pas sujette au vieillissement, possédant une structure granulaire allongée et ayant une valeur Rₘ égale au moins à 2,0.
